

July 7, 1959

G. A. RICHTER ET AL

2,893,754

SPECIAL PAPERS

Filed Feb. 29, 1944



Inventors  
George A. Richter &  
Arthur B. Lamb

By

J. J. T. *John T. Tracy*

Attorney

1

2,893,754

## SPECIAL PAPERS

George A. Richter, Rochester, N.Y., and Arthur B. Lamb, Cambridge, Mass., assignors to the United States of America as represented by the Secretary of the Navy

Application February 29, 1944, Serial No. 524,476

5 Claims. (Cl. 281—38)

The present invention relates to the manufacture of sheet material and more particularly to a special paper suitable for the preparation of readily "destructible" documents.

Broadly speaking, the object of the present invention is to provide a sheet material suitable for the preparation of documents that may be rendered unintelligible or indecipherable, merely by contacting the document with water.

A more particular object is to provide a paper of such a nature that any indicia or characters that have been written, printed or otherwise inscribed thereon become illegible when the document is immersed in any aqueous medium, including sea water.

A further object is to devise a book assembly so designed that water will rapidly reach all parts of every page when the assembly is immersed in water, and bring about the obliteration of all characters, patterns or indicia that may be marked on the individual pages.

Still another object is the provision of a new and improved process of fabricating "water-destructible" documents such as cipher key lists, code books, code strips and the like.

Other objects and advantages will be apparent as the invention is hereinafter more particularly described in connection with the two figures of the drawing wherein:

Fig. 1 is a perspective view of a bound volume; and Fig. 2 is a similar view of an unbound assembly, both in accordance with the present invention.

As a result of an extended investigation it has been found that the foregoing objects may be accomplished by utilizing a special type of sheet material provided with a special coating as hereinafter more particularly described.

The sheet material utilized in accordance with the present invention is characterized by the fact that, when uncoated surfaces thereof are pressed together and the assembly submerged in an aqueous medium, water will rapidly travel between the opposed surfaces, reaching all areas thereof in a relatively short period of time, and thence rapidly pass through the sheet to the opposite surface thereof. Sheet material of the foregoing type is coated with an oil-impervious, water-dispersible colloidal film-forming material. The resulting sheets are then utilized for the preparation of documents that may be rendered completely indecipherable by submersion in any aqueous medium, including sea water.

Numerous sheet materials are available today that possess the characteristics described above. In general, it has been found that such sheet materials are further characterized by a high degree of lateral expansion when wetted, and this latter property provides a convenient method of selecting a suitable sheet material for the construction of documents in accordance with the present invention. Of the available types of sheet material having a "high-lateral-wet-expansion," one of the most satisfactory materials is vegetable parchment. This may be

2

fabricated by any of the conventional methods, for example by treating a water leaf paper in the usual manner with relatively strong sulfuric acid for a short period of time, followed by thorough removal of the acid by a water-washing operation.

For purposes of the present invention, a high degree of parchmentization is desirable in order to insure "high-wet-expansion" and to favor great resistance to penetration by colloids when deposited from aqueous media.

10 Thus the percentage increase in sheet dimensions when a parchment sheet of the foregoing type is wetted, is from 10 to 20 times greater than the increase observed in the case of papers of the usual bond and ledger types. It should be understood, however, that other sheet materials having similar properties may be used, including glassine papers, vulcanized papers and regenerated cellulose such as that now marketed under the name "cellophane." However, for most purposes, parchment papers provide the most satisfactory and most readily procurable base for the improved "destructible" paper of the present invention.

A large number of materials are available that can be used to form the colloidal, oil-impervious, water-dispersible film with which the base sheet is coated. One of the 25 most satisfactory of these film-forming materials thus far discovered comprises water-soluble hydroxyethyl cellulose. Another material which serves substantially as well is low viscosity, water-soluble polyvinyl alcohol. Still other types of oil-impervious, water-dispersible colloidal coating materials may be employed where desired, particularly if they are applied to the base with a greater coverage than is found necessary with the preferred material (soluble hydroxyethyl cellulose). Thus one may employ gelatinous, water-soluble starches; water-soluble cellulose esters (e.g., partially hydrolyzed cellulose acetate); sodium borophosphate resins and the like.

Because of the colloidal nature of the gel produced when coatings of the foregoing type are wetted, any indicia that have been printed, inscribed or otherwise marked thereupon with an oil-base ink, are not only displaced laterally when the document is submerged in water, but also are individually disintegrated. Indeed the rate of disintegration effected by the viscous colloid is much more rapid and more complete than would be effected by a non-colloidal film. For the foregoing reasons, it is especially desirable to employ colloidal film-forming materials of the character described.

In order to give the coated paper a surface characterized by desirable handling properties, it may be advantageous in some instances to incorporate conventional secondary materials such as fillers, plasticizers, and the like, with the coating composition. The fillers add "tooth" to the surface, while the plasticizers tend to prevent hardening and embrittlement of the sheet under conditions of low humidity. In such cases, the customary types of fillers, plasticizers, etc. heretofore employed in the paper making art may be mentioned as representative of these two types of secondary materials.

For reasons explained hereinafter, where the ultimate object is to produce a book-like assembly, the "high-wet-expansion" sheet material is preferably coated with the water-dispersible film, on only one side of the paper. In any event, the coating operation may be satisfactorily accomplished by means of any of the conventional applicator devices such as those commonly used in the coated paper industry. The depth of the water-insoluble coating may be controlled by regulating the concentration of the coating mixture, the temperature, the viscosity, the setting of the brush applicator, or in any other suitable manner. The spreading can be accomplished by means of scraper blades or other conventional devices.

After the sheet material has been coated in the manner

described above it may then be dried. However, immediately following the coating operation, and before the evaporation of substantial proportion of the water, it is desirable to effect a "quick-set" of the gel in order to minimize penetration of the colloid into the sheet during the final drying operation. Such quick setting may be accomplished by a variety of means, e.g., by the use of infra-red rays, or by impinging a blast of hot air against the liquid film before substantial drying is brought about, or by quickly reducing the temperature of the colloid, thereby partially congealing the film. The sheet is then dried, preferably calendered and cut to suitable size.

The sheets prepared in the manner described above may be utilized in various ways for the production of "water-destructible" documents. Thus, for example, where the ultimate document is to consist of a single leaf or a number of loose leaves, the sheets may be coated either on one surface or on both surfaces with the water-dispersible film. The information is then printed, inscribed or otherwise marked upon the outer surface of the film, using an oil-base ink. Because of the oil-impervious nature of the coating, the indicia or characters utilized for the transmission of the information will be supported upon the outer or exposed surface of the water-dispersible colloidal film. Accordingly, when the document is wetted with an aqueous medium, the film is converted to a gelatinous, slimy, viscous liquid, the nature of which is such that the indicia are not only displaced laterally over the surface of the base sheet but they are also individually disintegrated, thereby rendering the document completely and permanently indecipherable.

Where the ultimate document is to consist of several leaves more or less tightly compressed together (as for example in the case of a bound volume), it is preferable to employ a method of assembly which will insure that water will reach all areas of every page when the document is immersed in an aqueous medium. To this end, the assemblies described hereinafter are particularly desirable inasmuch as they take full advantage of the fact that water will travel laterally between opposed uncoated surfaces of the special base sheet, much more rapidly than between opposed surfaces of ordinary paper stock, or between opposed coated surfaces of the special base sheet. For this reason, the preferred assembly for documents consisting of several leaves more or less compressed together, is constructed from a plurality of sheets of high-wet-expansion paper, each of which has been coated only on one surface with a water-dispersible, oil-impervious colloidal film. The "singly-coated" sheets are then assembled in accordance with either of the procedures described hereinafter.

According to the first method of assembly (Fig. 1), the indicia 3 for the transmission of the information are written, printed or otherwise inscribed upon the outer surface of the water-dispersible film, using an oil-base ink. The resulting leaves 4 and 5 are then assembled into book form in such a manner that the coated surface 6 of each leaf is in face-to-face relation with the coated surface of the adjacent leaf. When the resulting volume is immersed in an aqueous medium, the water rapidly passes between the opposed uncoated surfaces 7 of the individual leaves and thence penetrates through the sheet, converting the coating on the opposite surface to a viscous, gelatinous liquid that brings about the disintegration of the indicia imprinted on the coated surface.

An alternative method of constructing a document is of particular utility in preparing unbound documents wherein one or more sheets are placed in an envelope, folder or other container. The method, however, is also applicable to the preparation of a bound volume. According to this alternative method (diagrammatically shown in Fig. 2), coated special sheets 8 of the character described above, are employed as "bleeder elements" which are placed against the indicia-bearing sides of another sheet 9. In this case, the indicia-bearing page 10

consists of a bare sheet 11 (prepared either from any suitable paper stock or from parchment) that has been coated with a similar water-dispersible, oil-impervious colloidal film, the information being imprinted with an oil-base ink upon this film. The "bleeder element" consists of two opposed leaves 8 of high wet expansion paper coated only on the surfaces 12 which are unopposed to each other, the coating likewise consisting of a water-dispersible, oil-impervious colloidal film. It will thus be seen that the coated surfaces of the "bleeder element" are in face-to-face relation with the printed and coated side of the indicia-bearing pages. Even when the resulting assembly or any assembly prepared from a multiple of such elements, is compressed or folded together in booklike form and either bound or enclosed in a perforated envelope or other water pervious container, water will rapidly travel between the opposed uncoated surfaces 13 of the "bleeder element," thence pass through the pervious base sheet of the "bleeder element" and produce a slimy, viscous liquid not only from the water-dispersible film on the reverse face of the "bleeder element" but also from the corresponding film on the contacting surface of the indicia-bearing page. Any printed matter disposed on the film covering the indicia-bearing page will become disintegrated in the resulting viscous, gelatinous liquid.

Although any of the conventional oil-base inks may be employed in preparing the documents, it has been found that certain inks having a tendency to harden on aging, produce printed letters which take on the character of a film. Although such film-like characters are lifted from the sheet surface when the coating becomes jellied, they may sometimes retain their full structure even though they may be greatly displaced. When this occurs the result may be characterized as "alphabet soup." It is, therefore, preferable to employ inks which exhibit much less tendency for the retention of full letter structure and in such instances, there appears to be a strong tendency for the printed characters to break into small sections or portions and, therefore, to become more completely disintegrated.

In order to assure still more complete illegibility when the document is immersed in water, segmented lettering may be employed in preparing the document. Such lettering may be produced, for example, by the use of photographic screens or by other devices capable of producing letters consisting of a multiplicity of small dots. Segmented characters disperse much more readily and bring about a complete scrambling of the information.

In order to describe the nature of the present invention still more clearly, a specific example will herein-after be described in considerable detail. It should be clearly understood, however, that this is done solely by way of illustration and is not to be construed as a limitation upon the spirit or scope of the appended claims.

55

#### Example

In the following procedure, a parchment paper is selected as a preferred "wet expansion" paper. Such parchment paper is readily available in the form of rolls from various parchment paper producers, including the Paterson Parchment Paper Company, the Kalamazoo Vegetable Parchment Company and other sources.

The coating mixture described below is prepared and then applied continuously to one side of the sheet as it travels progressively past the applicator device. The rate of sheet travel will, of course, depend upon the apparatus employed and upon the capacity of the drying chamber into which the sheet is delivered following the application of the coating. Ordinarily, however, linear speeds of 20 to 100 feet per minute are practical.

The coating composition preferably consists of approximately a 5 to 10% solution containing the water-soluble, film-forming material, fillers, plasticizers, etc.

70

75

The following coating solution has been found very satisfactory:

|                                      | Percent |
|--------------------------------------|---------|
| Water-soluble hydroxyethyl cellulose | 4.8     |
| Cellite (Johns Manville type 352)    | 1.2     |
| Glycerin (95% c.p.)                  | 1.2     |
| Starch                               | 1.2     |
| Water                                | 91.6    |

The water-soluble hydroxyethyl cellulose may be obtained from Carbide and Carbon Chemicals Corporation, and as received usually consists of an aqueous solution containing 10% solids. In preparing the coating solution, water is added to the hydroxyethyl cellulose solution as received, in an amount sufficient to bring the concentration down to 7.5% solids. Thereafter the starch and Cellite, both dispersed in water, are added to this solution. The resulting mixture is passed through a colloid mill to break up any agglomerates. Finally, the glycerin is added to the homogenized solution. Violent agitation is to be avoided in order to minimize the foaming tendency. All steps in the preparation of the solution may be carried out at room temperature.

It is to be noted that because of the nature of the parchment and also because of the relatively high viscosity of the coating mixture, there is comparatively little penetration of the coating ingredients into the sheet, and every effort is preferably made to hold the coating mixture on the surface. The coating may be applied to the paper by means of a cloth application roll and smoothed by a series of vibrating brushes. The amount of coating is controlled by the pressure of the application belt on the paper. Control determination of the dry weight added to the paper may be made at the coating end. A weight increase of 3.5 lbs. per 1000 sq. ft. has been found quite satisfactory.

It is also desirable to direct continuous jets of steam against the uncoated side at the edge of the paper. This prevents the edge of the sheet from curling under, as happens when parchment is wetted on one side only.

The paper leaving the coating end of the applicator is preferably given a quick-set by means of infra red irradiation and blasts of hot air. Thereafter the sheet is dried continuously by hot air, care being taken to avoid over-drying, inasmuch as over-dried parchment is brittle and hard to handle during calendering. The dryer may consist of a large diameter heated roll upon which the uncoated side of the paper rests. If preferred, however, the drying operation may be carried out by means of hot air and by the use of a so-called festoon dryer. In either case, provision is made to have sufficient drying capacity to take care of the evaporation of the water. The sheet emerges from the drying chamber and is preferably reeled.

Where it is desirable to smooth the sheet surface or to improve the printability of the coated side, the paper is calendered. It has been found, however, that a high gloss on the face of the sheet produces a paper which sticks to the rubber blanket customarily employed in a multilith printing operation. Accordingly, the paper is preferably calendered with high pressure on the back of the sheet, thereby maintaining a semi-mat finish on the face. The coating and backing of the product may be carried out in any convenient manner. The roll of paper is cut into large sheets, and each sheet may be inspected and sorted for defects. The good sheets may then be square-cut into the required sizes without any further sorting. The culled sheets are also cut to smaller size and these are further inspected and sorted.

With the hydroxyethyl cellulose coating mixture, it has been found that a coverage of from about 2.5 to about 3.5 lbs. of coating solids per 1000 sq. ft. of paper produces a satisfactory product. The concentration, however, may be adjusted to meet any specified con-

ditions. The ratio of hydroxyethyl cellulose, filler and glycerin may be adjusted, and indeed may desirably be frequently changed in order to take care of slight differences which may occur in the base paper itself. The 5 filler may be starch, solid or powdered cellulose, talc or any equivalent material.

In fabricating a book assembly containing secret information, the photolithographic printing process is particularly satisfactory, especially where it is desired to produce individual letters or characters consisting of a multiplicity of small dots. As previously indicated, it is also preferable to employ an oil-base ink which has little tendency to harden by oxidation.

In assembling the leaves into a book form, the coated and printed surfaces 6 of successive leaves may be placed face to face as shown in Fig. 1. It may then be bound in any suitable manner, the page arrangement specified rendering it unnecessary to resort to special binding procedure. When the resulting book is immersed in sea water, the water rapidly passes between the contiguous uncoated faces 7 of the individual parchment sheets and thence penetrates through the sheet, dissolving and/or gelling the coating on the opposite surface thereof. Even when the sheets are tightly packed together in the form of books or pamphlets, because of the colloidal nature of the resulting film, the obliteration of the indicia on the sheets is remarkably rapid and the information contained on the page becomes unintelligible.

A satisfactory production control test may be carried out to determine the destructibility of the document. Thus, for example, a small 2" square book of 50 pages may be bound between two perforated metal plates and the assembly placed in a tray under an applied pressure of 20 grams per sq. cm. A 3% salts solution is then poured into the tray covering the booklet to a depth of 6". At the end of 1½ hours to 5 hours the book is removed and inspected. The printing on a satisfactory sample will be thoroughly disintegrated at the end of that time.

40 In view of the foregoing detailed description it will be apparent to those skilled in the art that many modifications may be made without departing from the spirit of the invention. All such modifications are to be understood as included within the scope of the invention as defined in the appended claims.

45 We claim:

1. An assembly of the character described, including at least one indicia-bearing page, a bleeder element, said indicia-bearing page positioned in contact with said bleeder element, said indicia-bearing page comprising sheet material having a water-dispersible, oil-impervious colloidal film thereon adapted to support said indicia on the outer surface of said film; said bleeder element comprising at least two opposed leaves of sheet material having a high-wet-expansion, coated only on the surfaces which are unopposed to each other, with a water-dispersible, oil-impervious colloidal film adapted to contact the corresponding film on an adjacent indicia-bearing page.

2. An assembly of the character described composed of 60 at least one pair of leaves of sheet material having consecutive indicia-bearing pages, a bleeder element, said indicia-bearing pages separated from each other by said bleeder element disposed therebetween, said indicia-bearing pages having a water-dispersible, oil-impervious colloidal film thereon adapted to support said indicia on the outer surface of said film; said bleeder element comprising at least two leaves of sheet material having a high expansion when wetted, coated only on the surfaces which are unopposed to each other with a water-dispersible, oil-impervious colloidal film and disposed to contact the corresponding film on an adjacent indicia-bearing page.

3. A document of the character described, including a base sheet of cellulosic material having a high-wet-expansion; a water-destructible oil-impervious, colloidal coating on at least one surface of said sheet, and inked indicia,

comprising segmented printed characters, upon the outer surface of said coating.

4. A book assembly comprising a plurality of leaves of cellulosic sheet material of high-wet-expansion, said leaves being coated on at least one surface with a water-dispersible, oil-impervious, colloidal film, inked indicia, comprising segmented characters, being disposed on the outer surfaces of said water-destructible film.

5. A book assembly comprising a plurality of leaves of cellulosic sheet material of high wet-expansion bound together, said leaves being coated on one surface only with a water-dispersible oil-impervious colloidal film and arranged so that the coated surface of each leaf is in face-to-face relation to the coated surface of an adjacent leaf,

10 and inked disintegratable indicia disposed on the outer surface of said water-destructible film.

**References Cited in the file of this patent**

**UNITED STATES PATENTS**

|           |                 |                |
|-----------|-----------------|----------------|
| 171,871   | Schnoble        | Jan. 4, 1876   |
| 2,225,520 | Eisenberg       | Dec. 17, 1940  |
| 2,235,798 | Collings et al. | Mar. 18, 1941  |
| 2,240,999 | Moreton         | May 6, 1941    |
| 2,285,490 | Broderick       | June 9, 1942   |
| 2,300,787 | Inglass         | Nov. 3, 1942   |
| 2,322,887 | Schwartz        | June 29, 1943  |
| 2,359,185 | Wysong          | Sept. 26, 1944 |